

May 13, 1947.

O. H. LEIDY

2,420,604

ADHESIVE WRAPPING TAPE

Filed July 9, 1945



INVENTOR.

Orris H. Leidy.

BY

Harness, Dickey & Pierce.

ATTORNEYS.

## UNITED STATES PATENT OFFICE

2,420,604

## ADHESIVE WRAPPING TAPE

Orvis H. Leidy, Grosse Pointe, Mich., assignor  
to Michigan Chrome & Chemical Company,  
Detroit, Mich., a corporation of Michigan

Application July 9, 1945, Serial No. 603,955

3 Claims. (Cl. 154—53.5)

1

This invention relates generally to protective electrolytic or dielectric coating materials. More particularly, it relates to a novel and improved form of dielectric tape primarily designed and intended for use in electroplating or electrolytic operations.

While the primary use of tapes or materials of this general category is for masking electroplating racks, it will be readily appreciated that the improvements of the present invention will find utility in the masking of parts to be plated and for other similar purposes in connection with the electrodeposition of metals and electrolytic pickling and cleaning operations.

Since the function of electrolytic protective coatings of the general character to which the present invention relates is to mask or coat portions of an article or element to be submerged in an electrolytic bath, it is of primary importance that the coating applied effectively cover and seal those portions of the article which it is desired to protect. In order to accomplish this, the present invention contemplates the provision of an electrolytic coating material in the form of a substantially homogeneous, resinous, ribbonlike tape which is preferably of considerably thinner dimension in its side marginal edge portions than it is in its central portion whereby to provide a sort of feather edge structure which is particularly effective in obtaining a tight seal with respect to the article to which the tape is applied.

Generally speaking, rubber and rubberlike materials have been widely used as protective coatings in operations of this general character and have been widely used for this purpose. However, it has been found that protective coatings formed in accordance with the teachings of the present invention are considerably easier to apply, provide a tighter seal and not only have physical characteristics substantially equivalent to those of rubber, but at the same time have very superior chemical characteristics when intended for use in a wide variety of baths or solutions.

The coating structure formed in accordance with the teachings of the present invention offers effective resistance and complete protection when used in conventional plating solutions throughout all operating temperature ranges. This is particularly important when the coatings of the present invention are applied to plating racks or used as masking for articles being plated, inasmuch as the racks and the articles may be exposed to extremely hot cleaning and pickling solutions, as well as to plating baths which may

2

range from high acid baths to highly alkaline baths.

Still further, the present invention contemplates the provision of an electrolytic coating which, when applied, not only has high dielectric strength, but which inherently provides a relatively smooth, glossy coating. This feature is important as in electrolytic operations it allows more thorough rinsing and drainage, thereby reducing the dragout of solutions.

Still further, the invention contemplates the provision of a substantially homogeneous, resinous, ribbonlike tape which has relatively high tensile strength, thereby permitting easy application, tight wrapping of the portions of the parts to be protected without tearing or breaking.

Still further, the invention contemplates the provision of a protective tape which, while relatively smooth and glossy in appearance and while not tacky or sticky to touch, effectively adheres and sticks to itself when tightly wrapped around the articles to be protected.

Many other and further objects, advantages, and features of the present invention will be come more clearly apparent from the following specification, the drawings relating thereto, and from the claims hereinafter set forth.

In the drawings:

Figure 1 illustrates a fragmentary portion of 30 the plating rack having portions thereof protected by the application of the improved electrolytic tape in accordance with the teachings of the present invention.

Figure 2 illustrates in perspective a roll of the 35 tape as produced for providing such coatings.

Figure 3 is an enlarged cross-sectional view of 40 tape formed in accordance with the teachings of the present invention, illustrating the preferable cross-sectional configuration of the improved coating material.

With more particular reference to the drawing, it will be readily appreciated that in order to be effective for the purpose intended, tape of the general character to which the present invention 45 relates must be relatively flexible, elastic, and be capable of substantial adherence to itself or to the articles being covered without being sufficiently gummy or tacky to prevent satisfactory handling. Consequently, the material from 50 which the tape of the present invention is formed and its manner of fabrication constitute important features of the present invention.

While many of the advantageous features of 55 the present invention may be employed by the substitution of various other resinous materials,

for the specific composition hereinafter set forth, it has been found preferably to produce the tape of the present invention by extrusion of an appropriate mixture of resinous material through a conventional extrusion die into an appropriate bath of coagulating fluid. Such extrusion operations are well known and any conventional method may be employed.

The improved tape is preferably formed of a copolymer of two different vinyl compounds, by which is meant the conjoint polymerization of two or more compounds while in mutual contact. One of these compounds comprises a vinyl halide such as vinyl chloride, for example, or vinyl benzene (styrene), this compound being generally known as "hard" resin, and the other compound is preferably an ester of a lower aliphatic acid such as vinyl acetate, vinyl propionate, or vinyl butyrate, for example, generally referred to, when separately polymerized, as "soft" resin.

When two such resins are conjointly polymerized and the resultant product extruded to form a substantially continuous tape, the resultant product has been found to be particularly useful for dielectric protective coatings such as are required in electroplating operations. Patent No. 2,072,170, dated March 2, 1937, to George K. Herzog, describes the utilization of copolymers of these resins and their use for sprayed coatings in chromium plating tanks. As is set forth in this patent, the tape of the present invention is preferably produced by using 50 to 95 parts of the vinyl compound of the "hard" resin-forming type, and 50 to 5 parts of the vinyl ester of the "soft" resin-forming type, it being found preferable to utilize as a general rule approximately 93 to 95 parts of "hard" forming type resin and 7 to 5 parts of "soft" forming type resin.

When appropriate proportions of these two types of resins are copolymerized and extruded through an extrusion die to provide a cross-sectional configuration to that shown in Figure 3 of the drawing, a particularly satisfactory product results. The resultant product has a generally glossy appearing finish and is not sticky or tacky to handle, is easily and conveniently applied to plating racks or parts to be plated, and provides a particularly effective coating covering. This is particularly true because of the fact that the tape has a relatively high tensile strength and considerable resilience and, therefore, can be tightly wrapped around and engage the surface of the parts to be protected to provide a protective coating and at the same time effectively adhering to itself in order to provide a substantially continuous coating over the surface to which the tape is applied.

While not essential to provide an adequate protective covering, it is in some instances desirable to bake or heat-treat the wrapped coating after the same has been applied. This baking serves to fuse adjacent portions of the tape together and to a certain extent provide a tighter and more effective seal.

While the particular dimensions of the cross-sectional configuration of the tape may be varied throughout a relatively wide range and yet at the same time obtain satisfactory results, it has been found that for a tape of approximately three-fourths inch in width, the tape should be approximately .012" thick in its central portion, tapering to perhaps a thickness somewhat less than

.005" at its marginal edges, thereby providing a generally feathered edge structure particularly effective in obtaining a tight seal when applied to the surface of a part to be covered or to other portions of the tape itself.

Many modifications may be made in the improvements herein described without departing from the spirit and scope of the invention as set forth in the following claims.

What is claimed is:

1. An electrolytic protective flexible elastic tape comprising a generally homogeneous resinous ribbon-like strip having a generally glossy surface adherent to itself but yet capable of satisfactory handling and having a tensile strength sufficient for tight wrapping of the tape without breaking or tearing, said tape being of substantially greater thickness in its central portion than at its marginal edges whereby, when applied to and maintained under tension on an article to be treated and subsequently heat treated, there results a fusing together of adjacent portions of the tape in order to provide a tight and effective seal while retaining the tensile strength in the thicker portion of the tape.

2. An electrolytic protective flexible elastic tape comprising a generally homogeneous resinous ribbon-like strip having a generally glossy surface adherent to itself but yet capable of satisfactory handling and having a tensile strength sufficient for tight wrapping of the tape without breaking or tearing, said tape being of maximum thickness in its central portion and tapering to substantially a feather edge at its marginal edges whereby, when applied to and maintained under tension on an article to be treated and subsequently heat treated, there results a fusing together of adjacent portions of the tape in order to provide a tight and effective seal while retaining the tensile strength in the thicker portion of the tape.

3. An electrolytic protective flexible elastic tape comprising a generally homogeneous resinous ribbon-like strip having a generally glossy surface adherent to itself but yet capable of satisfactory handling and having a tensile strength sufficient for tight wrapping of the tape without breaking or tearing, said tape being of maximum thickness in its central portion and gradually tapering to a substantially reduced thickness at its marginal edge portions whereby, when applied to and maintained under tension on an article to be treated and subsequently heat treated, there results a fusing together of adjacent portions of the tape in order to provide a tight and effective seal while retaining the tensile strength in the thicker portion of the tape.

ORVIS H. LEIDY.

#### REFERENCES CITED

The following references are of record in the file of this patent:

#### UNITED STATES PATENTS

| Number    | Name       | Date          |
|-----------|------------|---------------|
| 1,357,350 | Schumacher | Nov. 2, 1920  |
| 2,105,728 | Geller     | Jan. 18, 1938 |
| 2,101,876 | Scott      | Dec. 14, 1937 |

#### OTHER REFERENCES

Pamphlet, Vinylite Resins, Carbide and Carbon Chemicals Corp., May 1, 1937, page 6. (Copy in Division 50.)